

# UNITED STATES PATENT OFFICE.

EDWARD D. GLEASON, OF NEW YORK, N. Y., ASSIGNOR TO FRANK JOHN ROESLER, OF BROOKLYN, NEW YORK.

## COPPER-ALUMINUM ALLOY.

1,076,973.

Specification of Letters Patent.

Patented Oct. 28, 1913.

No Drawing.

Application filed October 22, 1912. Serial No. 727,107.

*To all whom it may concern:*

Be it known that I, EDWARD D. GLEASON, of Brooklyn, in the county of Kings, city and State of New York, have invented a 5 certain new and useful Improvement in Copper-Aluminum Alloys, whereof the following is a specification.

My invention relates to alloys the principal ingredient of which is copper, and an 10 object thereof is to provide such alloys including a given percentage of copper but of different degrees of hardness.

In practising my invention I incorporate boron in aluminum, as graphite exists in 15 cast iron, by fusing them in a crucible, free from impurities, with a flux consisting of native calcium fluorid and fused vitrified boracic acid. For instance, in a crucible of magnesite, or graphite free from arsenic 20 balls; I put three parts of calcium fluorid and on top of that, one part of fused vitrified boracic acid. I then fuse the same, preferably in an oxyhydrogen furnace of ordinary commercial type, until the fused 25 mass of said two ingredients has reached the proper consistency; which is manifested by dense fumes of boron fluorid arising from the crucible. I then inject into the fused mass pure aluminum in ingot form.

As aluminum melts at a comparatively low 30 temperature, it fuses and absorbs the gases freed from the other ingredients. When said mass is fused, the molten aluminum is between two layers of boron fluorid, the top 35 layer acting as a cover preventing oxidization, while the lower layer mixes with the molten aluminum. Thereupon, I cast the mixture of calcium fluorid, fused vitrified boracic acid and pure aluminum as ingots; 40 the mass being well stirred and allowed to stand for a few minutes, in the crucible, before being poured. I then melt 90 parts of pure copper, in a crucible, under a cover of charcoal and black oxid of manganese, 45 and while the copper is at high temperature I add thereto an amount slightly in excess of 10 parts of the boron aluminum product aforesaid.

It may be observed that in the ordinary 50 foundry practice of making aluminum

bronze, there is a rise in temperature upon the inclusion of the aluminum in the fused copper, which does not occur in practising my invention aforesaid, and the product of my invention has entirely different characteristics from those of ordinary aluminum bronze. For instance, aluminum *per se* has 55 the property of absorbing a large percentage of oxygen, forming aluminum oxid, and, when ordinary aluminum bronze is 60 rolled to form sheets or drawn to form wire, the oxid of aluminum appears as minute black spots in said products resulting in the commercial failure thereof. On the contrary, no aluminum oxid appears with my 65 improved alloy, for the reason that boron in combining with aluminum removes the oxygen and dissolved gases, and, my aluminum boron alloy aforesaid, containing boron in excess, removes the dissolved gases 70 and oxygen from the copper, when combining with the latter. Moreover, a trace of metallic manganese is left in the copper from the cover and flux of black oxid of manganese and facilitates the deoxidizing 75 effect aforesaid; so that rolled sheets of my improved alloy are found to be free from aluminum oxid upon microscopic inspection.

My improved alloy may be made in any 80 desired degree of hardness with the same percentage of copper by adding aluminum with more or less boron; the different degrees of hardness being readily manifested by a Shore scleroscope. For instance, my 85 improved alloy consisting of 90 parts copper and 10 parts boron aluminum may be made so hard as to be advantageously employed in the manufacture of edge tools; said alloy being capable of being forged 90 into hatchet heads, etc., or, rolled hot into sheets from which blades for knives or safety razors may be formed; it being characteristic of said alloy that it resists corrosion, and the action of acids to a limited 95 degree, and holds its edge as well as steel.

I do not desire to limit myself to the precise methods of procedure or proportions herein set forth as it is obvious that various modifications may be made therein without 100

departing from my invention as defined in the appended claims.

I claim:

1. An alloy consisting of boron, copper and aluminum.
2. A process consisting of fusing calcium fluorid and vitrified boracic acid and adding aluminum thereto; and, adding the mixture of said three ingredients to molten copper.
3. An alloy consisting of 90 parts copper 10 and 10 parts of boron aluminum.

In testimony whereof, I have hereunto signed my name, at Brooklyn, New York, this nineteenth day of October, 1912.

EDWARD D. GLEASON.

Witnesses:

HENRY J. MEYER,  
BENJAMIN ZEKOWSKI.